

3,505,130  
**METHOD FOR IMPROVING FATIGUE STRENGTH  
IN TURBINE BLADES**  
William Douglas Paul, Caledon, Ontario, Canada, assignor, by mesne assignments, to Orenda Limited, Toronto, Ontario, Canada, a company

No Drawing. Filed May 29, 1967, Ser. No. 642,135  
Claims priority, application Great Britain, June 13, 1966,  
26,308/66

Int. Cl. C21d 7/00; C21f 1/00; B24c 1/10  
U.S. Cl. 148—11.5 9 Claims

## ABSTRACT OF THE DISCLOSURE

A method for treating turbine blades fabricated from high temperature alloys involving two cold working operations on the surfaces of the blades and a heat treatment between the cold working operations whereby a substantial increase in the strength of the blades is achieved.

## BACKGROUND OF THE INVENTION

The production of highly-stressed machine components usually involves considerable machining of forgings, wrought billets and the like. Generally speaking, the forging process gives better grain structure and improved physical properties of the material than do other processes. However, the increased machining required to produce the finished article results in greater production costs. Casting methods on the other hand have improved to such an extent that much less machine finishing is needed. The casting process, though, is still not conducive to the formation of the fine-grain structure giving properties similar to those of forged products.

Grain size in castings can be reduced somewhat by controlling the cooling rate of the casting in the mould, but this is not a precise or easy method and varies in effectiveness with the size and intricacy of the casting. Another method used to maintain fine grain size is that of introducing inoculants into the melt. Inoculants work reasonably well with investment castings and particularly with small castings where casting temperatures can be kept relatively low. With more massive castings the inoculation method becomes less effective, presumably because the inoculants dissolve in the molten metal before solidification begins.

Cold working by processes such as shot-peening and cold rolling can, by introducing residual compressive stresses in the surface of a cast or wrought material, improve the fatigue strength and, in some cases, decrease susceptibility to stress corrosion. Cold working by itself, however, has been found not to yield these results uniformly with all materials, particularly in some of the cast super-alloys such as Inconel 713. Components which depend on residual stresses for improvement of fatigue strength may be used only where operating temperatures are not high enough to cause relief of the residual stresses.

It is well known that certain materials, such as some of the nickel-base group, which have had their surface layers cold worked and have then been heat-treated at a temperature sufficient to cause re-crystallization into a fine-grain structure at the surface, have improved fatigue strength. In U.S. Patent No. 2,920,007 to B. O. Buckland a turbine blade for high temperature use is described which is cold worked to harden the surface of the metal to a depth of several mils. The patent teaches that the surface layer of the blade is then re-crystallized by heat treatment to a small grain size to improve the rupture and fatigue resistant properties of the outer protective layer. However, the alloys referred to in this patent are

wrought alloys, having been used as turbine blades only in the form of forgings. The procedure described in this patent is not nearly as successful with investment cast turbine blades. In any case, the treatment of wrought turbine blades in accordance with the teachings of this patent does not increase the fatigue resistance of the blades to the extent which would be most desirable.

## SUMMARY

It has now been discovered that the step of cold working the surface of the turbine blade a second time, after the heat treatment which causes re-crystallization in the surface layer, further considerably increases the fatigue strength of the turbine material.

In the method of the invention turbine blades of alloys designed for elevated temperature service are first cold worked at their surface layers such as by machining or shot-peening. The blades being treated are substantially in the shape desired for use before shot-peening or in the desired shape after machining if the first cold working step is accomplished by machining. After the first cold working step the blades are heat treated at a temperature or temperatures sufficient to cause re-crystallization of the cold-worked surface layers into a fine-grained structure at the surface of the blades. The particular heat treatment depends of course on the particular alloy involved. After the heat treatment the blades are cold worked a second time at the surface thereof to further substantially increase the fatigue strength of the blades to re-introduce favourable residual stresses in the blades. The second cold working operation, not heretofore used in the art, which increases the turbine blade fatigue resistance to a considerable degree, is found, for example, to increase the fatigue resistance of superalloys, such as Inconel 713 alloy and Udiment 500 alloy, by in the order of 75%, an increase which is more than would be normally expected.

It is an object of the present invention to provide a procedure for substantially increasing the fatigue strength of turbine blades fabricated from high temperature alloys.

Other objects and advantages of the invention will be apparent from the following description of the preferred embodiments.

## DESCRIPTION OF THE PREFERRED EMBODIMENTS

A turbine blade processed according to the invention is advantageously subjected first to preliminary heat treatment operations to improve the mechanical properties thereof with any machining necessary, such as on the root structure, being carried out. The first cold working operation on the surfaces of the blade is then carried out with such cold working being necessary only on all sides of the root stem of the blade below the root platform thereof where improved fatigue resistance is particularly required. As afore-described shot-peening, carried out in accordance with techniques well known to the art, is an advantageous way of cold working the surfaces of the blades although machining of the surfaces also accomplishes this end. After the blade has been heat treated to cause re-crystallization of the cold-worked surface layers into a fine-grained structure, the final cold working operation on the surface layers of the blade is advantageously carried out by way of a shot-peening operation in a manner similar to and in the same area as the first shot-peening operation.

The process of the invention is particularly attractive for components such as investment cast turbine blades and the like which are made from high-temperature super-alloys such as Inconel 713 alloy and Udiment 500 alloy since, in general, their hot strength is such that it is not

practical to break down the coarse-grained, cast structure by processes such as forging and rolling. Although in operation, gradual loss of the residual stresses introduced by the second cold working occurs in some parts of the blade, the service temperatures at the blade root, the critical area, are sufficiently low to ensure retention of the residual stresses over long periods. Notwithstanding the eventual loss of the residual stresses in the aerofoil area of the blade the fine-grain surface structure retains improved mechanical and thermal fatigue properties.

However, any blades fabricated from high temperature alloys which are work hardenable can be treated to advantage in accordance with the invention. Thus, even though a fine grain size is obtained at the surface of forged turbine blades of wrought alloys in accordance with prior art procedures, the three stage procedure of the invention involving first and second surface cold working operations with a re-crystallization heat treatment operation therebetween acts to improve the fatigue resistance of wrought turbine blades, fabricated from alloys such as, for example, Hastelloy "B," Crucible 422, Nimonic 80 and Inconel X alloys, since the larger grain size in the substrate or core of the wrought blade inhibits creep.

For the purpose of giving those skilled in the art a better understanding of the invention the following illustrative examples are given:

#### EXAMPLE I

A number of first stage turbine blades were investment vacuum cast from Udimet 500 alloy which is a nickel-base alloy containing 18% Cr, 18% Co, 4% Mo, 3% Al, 3% Ti and 2% Fe. The blades were given a standard heat treatment, first at 2100° F. for 4 hours in vacuum, followed by air cooling, and then heating for 2 hours at 1975° F. in vacuum, followed by air cooling. Four of the blades were then surface cold worked over the full root stem portion by machining and another four blades were cold worked on their surface, again over the root stem sections thereof, by shot-peening in accordance with well known procedures. All eight blades were then heat treated by first heating at 1975° F. in vacuum for 2 hours and then at 1400° F. in vacuum for 16 hours. This heat treatment resulted in re-crystallization of the surface cold worked layer into a fine-grained structure. Two of the blades subjected to cold working by machining and two subjected to cold working by the shot-peening were then subjected to a second cold working treatment on the surface layer thereof by shot-peening on the root stem sections in a manner similar to the shot-peening first carried out. The second shot-peening treatment was omitted for the other four blades.

All eight blades were then fatigue tested by holding the roots of the blade stationary in a fixture while driving the airfoils electromagnetically at increasing amplitudes. The tests were run for  $2 \times 10^6$  cycles at increasing amplitudes of 0.040", 0.044", 0.049", 0.054" and 0.060" until cracks developed, at which time a test was stopped. Thus, any one test was driven for  $2 \times 10^6$  cycles at each amplitude until cracks developed. The results of these tests are set forth in Table A following:

TABLE A

| Blade No. | First Cold Working | Second Cold Working | Final Amplitude Reached (inch) | Reversals at Final Amplitude |
|-----------|--------------------|---------------------|--------------------------------|------------------------------|
| 1.....    | Machined.....      | No.....             | 0.044                          | 1,734,600                    |
| 2.....    | do.....            | No.....             | 0.049                          | 1,366,800                    |
| 3.....    | Shot-peened.....   | No.....             | 0.054                          | 98,800                       |
| 4.....    | do.....            | No.....             | 0.054                          | 687,900                      |
| 5.....    | Machined.....      | Yes.....            | 0.080                          | 1,454,100                    |
| 6.....    | do.....            | Yes.....            | 0.060                          | 1,033,200                    |
| 7.....    | Shot-peened.....   | Yes.....            | 0.060                          | 462,500                      |
| 8.....    | do.....            | Yes.....            | 0.080                          | 1,599,840                    |

It is readily apparent from the results shown in Table A that the blades subjected to the final surface cold working treatment had considerably improved fatigue strength

over those blades not subjected to the second cold working treatment. The fatigue strength of the four blades treated in accordance with the invention are seen to have had uniform high fatigue strength, all of them withstanding  $2 \times 10^6$  reversals at the first four stress levels and well into the fifth stress level, whereas the blades partially processed, and not in accordance with the method of the invention, exhibited considerable scatter in properties with failures occurring in the second, third and fourth stress levels.

The operation of the method of the invention was also tested out on the nickel base Inconel 713 alloy. Specimens were tested for endurance strength (1) in the as cast condition, (2) as cast and shot-peened, (3) as cast and treated in accordance with the process of the invention (shot-peened, heat treated and shot-peened), and (4) as cast and then heat treated and shot-peened (the first step of the process being deleted). Heat treatment where carried out was the same as that used in Example I. The results of these tests are set forth in Table B following.

#### EXAMPLE II

TABLE B

| Test Series No. | Treatment                                | Endurance Strength (p.s.i.) | Comments                                        |
|-----------------|------------------------------------------|-----------------------------|-------------------------------------------------|
| (1).....        | As cast.....                             | 50,750                      | Average of four R. R. Moore tests. <sup>1</sup> |
| (2).....        | As cast and shot-peened.....             | 53,075                      | Average of four R. R. Moore tests.              |
| (3).....        | As cast and full three step process.     | <sup>2</sup> 63,760         | Average of three R. R. Moore tests.             |
| (4).....        | As cast, heat treatment and shot-peened. | 90,000                      | Average of two Cantilever beam tests.           |
|                 |                                          | 41,460                      | Cantilever beam tests.                          |

<sup>1</sup> The R. R. Moore is a well known fatigue test machine which employs a rotating beam test specimen.

<sup>2</sup> These R. R. Moore fatigue test results were considered to be in error on the low side since the high temperature heat treatment on these specimens caused a small amount of distortion producing unusually severe vibration during the rotating beam fatigue tests.

The specimens subjected to the full three step process of the invention had considerably improved fatigue strength over the as cast and the as cast and shot-peened specimens. There is also seen to be an impressive improvement over specimens treated to heat treatment and shot-peening from the as cast condition, with one shot-peening operation being deleted.

It can be seen that the method of the invention results in substantially improved fatigue properties in items fabricated from superalloys and used in elevated temperature service and in particular in turbine blades made from such alloys. It is found that the invention is useful for treating items made from any high temperature alloys which are work hardenable and it is found that the method of the invention can be used to advantage with wrought superalloys by permitting use of a higher-than-normal solution heat-treatment temperature. Though resulting in larger-than-normal grain size throughout the forging, it is possible to restore fine-grain structure at the surface, and thus the good, and in fact better, fatigue properties by the forging products in accordance with the invention.

What I claim as my invention is:

1. A method for increasing the fatigue resistance of turbine blades of work hardenable alloys designed for elevated temperature service, said blades having been formed to substantially the desired shape, which comprises first cold working at least part of the turbine blades only at their surfaces, heat treating the turbine blades at a temperature sufficient to cause recrystallization into a fine-grained structure at the cold worked surfaces of the blades and, after said heat treatment, cold working said blades a second time at the said surfaces thereof to increase the fatigue strength of the blades to a considerable degree.

2. A method as claimed in claim 1 wherein investment

cast turbine blades are treated to increase their fatigue strength.

3. A method as claimed in claim 1 wherein wrought turbine blades are treated to increase their fatigue strength.

4. A method as claimed in claim 1 wherein the first cold working operation is carried out by machining the turbine blade.

5. A method as claimed in claim 1 wherein the first cold working operation is carried out by shot-peening the turbine blade.

6. A method as claimed in claim 4 wherein the second cold working operation is carried out by shot-peening the turbine blade.

7. A method as claimed in claim 5 wherein the second cold working operation is carried out by shot-peening the turbine blade.

8. A method as claimed in claim 7 wherein shot-peening of the turbine blade is directed only on all sides of the root stem of the blade below the root platform thereof.

9. A method as claimed in claim 2 wherein the first

and second cold working operations are carried out by shot-peening the turbine blade and such shot-peening is directed only on all sides of the root stem of the blade below the root platform thereof.

#### References Cited

##### UNITED STATES PATENTS

|           |        |                     |            |
|-----------|--------|---------------------|------------|
| 2,560,973 | 7/1951 | Martin et al. ----- | 148—12     |
| 2,782,135 | 2/1957 | Richardson -----    | 148—11.5   |
| 2,920,007 | 1/1960 | Buckland -----      | 148—11.5 X |

##### OTHER REFERENCES

Metals Handbook, vol. 2, 1964, pp. 398—403, and 488.

15 L. DEWAYNE RUTLEDGE, Primary Examiner

G. K. WHITE, Assistant Examiner

U.S. Cl. X.R.

20 148—12, 39